

[54] FOGGED, DIRECT POSITIVE SILVER HALIDE EMULSION SENSITIZED WITH A NITROPHENYL MERCAPTO HETEROCYCLIC COMPOUND

2,947,629 8/1960 Stewart et al. .... 96/101  
3,615,607 10/1971 Soma et al. .... 96/101

[75] Inventors: **Keisuke Shiba; Masanao Hinata; Reiichi Ohi; Tadao Shishido**, all of Kanagawa, Japan

*Primary Examiner*—Won H. Louie, Jr.  
*Attorney, Agent, or Firm*—Sughrue, Rothwell, Mion, Zinn & Macpeak

[73] Assignee: **Fuji Photo Film Co., Ltd.**, Kanagawa, Japan

[57] **ABSTRACT**

[22] Filed: **Dec. 19, 1973**

A silver halide photographic emulsion for direct positives, containing at least one compound represented by the general formula (I),

[21] Appl. No.: **426,146**

[30] **Foreign Application Priority Data**

Dec. 19, 1972 Japan ..... 47-127575

[52] **U.S. Cl.** ..... **96/100**; 96/107; 96/108; 96/101

[51] **Int. Cl.<sup>2</sup>** ..... **G03C 1/28**

[58] **Field of Search** ..... 96/107, 108, 100, 101

[56] **References Cited**

UNITED STATES PATENTS

2,901,351 8/1959 Van Pee et al. ..... 96/101



in which Z represents a group of non-metallic atoms necessary for forming a heterocyclic ring and n represents an integer of from 1 to 3.

**26 Claims, No Drawings**

**FOGGED, DIRECT POSITIVE SILVER HALIDE  
EMULSION SENSITIZED WITH A NITROPHENYL  
MERCAPTO HETEROCYCLIC COMPOUND**

**BACKGROUND OF THE INVENTION**

1. Field of the Invention

This invention relates to a silver halide photographic emulsion and, more particularly, it is concerned with a silver halide photographic emulsion for direct positives containing a nitrophenylmercapto group-containing heterocyclic compound.

2. Description of the Prior Art

When a silver halide light-sensitive material is exposed to light with in the light-sensitive wavelength range of this light-sensitive material and developed, the blackened density increases and leads to a maximum value with an increase of the quantity of exposure, but decreases again and forms finally a positive image with a further increase in the quantity of exposure. Such a phenomenon is generally called "solarization." A similar reversal phenomenon is also found with a silver halide which as been fogged optically or chemically in the process of producing the silver halide emulsion to that by light. The expression "direct positive emulsion" or "emulsion for direct positive" as used throughout this specification is to be understood as an emulsion which is processed to form a positive image by ordinary exposure and development.

The instant invention relates to a direct positive emulsion sensitive to the blue color region by the incorporation of an organic densensitizer. For example, in U.S. Pat. No. 3,501,307 an emulsion of the type that is reversed by the use of an organic densensitizer such as pinakryptol yellow or 5-m-nitrobenzilidene rhodanine is disclosed. It is known that an emulsion fogged using a relatively small amount of a gold compound or salt and a reducing agent and containing at least 50 mol % of silver bromide can be advantageously used to obtain a particularly high reversal sensitivity and that an organic densensitizer is effective for the sensitization of such an emulsion. However, known organic densensitizers which have hitherto been used for the sensitization in the blue color region have various disadvantages.

In general, an organic densensitizer having a relatively high reversal sensitivity reduces the maximum density of an original emulsion, while, on the other hand, a sensitizing agent which does not reduce the maximum density gives only a low reversal sensitivity. In this specification, an organic densensitizer-free emulsion will hereinafter be referred to as an "original emulsion." For example, pinakryptol yellow reduces the maximum density of an original emulsion and colors a photographic material used yellow. 3-Ethyl-5-m-nitrobenzilidene rhodanine does not reduce the maximum density as much, but the clarity is bad, that is, the value of minimum density is large. 5-m-Nitrobenzilidene rhodanine

does not reduce the maximum density as much and the value of minimum density is small, that is, the clarity is good, but a lower reversal sensitivity is obtained. Therefore, it is very important to find an organic densensitizer for sensitizing in the blue color region, which is capable of giving a high reversal sensitivity without reducing the maximum density and with a high clarity.

It is a principal object of the invention to provide a silver halide photographic emulsion for direct positives, which contains an organic desensitizer for sensitization in the blue color region, capable of giving a high sensitivity, being substantially free from any residual coloring and without reducing the maximum density of an original emulsion.

**SUMMARY OF THE INVENTION**

The objects can be accomplished by the incorporation of at least one compound represented by the following general formula (I) in an original emulsion,

General Formula (I)



in which Z represents a group of nonmetallic atoms necessary for forming a heterocyclic ring and n represents an integer of from 1 to 3.

**DETAILED DESCRIPTION OF THE INVENTION**

Suitable examples of heterocyclic rings in the above described general formula are 1,2,4-triazole ring, a 1,3,4-thiadiazole ring, a 1,3,3a,7-tetrazaindene ring, a benzothiazole ring, a benzimidazole ring and a pyrimidine ring.

The heterocyclic ring formed by Z can be either a substituted ring or an unsubstituted ring. The particular substituent(s) on the ring is not important so long as the substituent(s) used does not deteriorate substantially the photographic properties in terms of sensitivity, residual coloring and maximum density.

Suitable examples of substituents include an alkyl group preferably having up to 20 carbon atoms (e.g.,  $\text{CH}_3$ ,  $n\text{-C}_5\text{H}_{11}$ ,  $n\text{-C}_9\text{H}_{19}$ ,  $n\text{-C}_{17}\text{H}_{35}$ , etc.), an aryl group (e.g., an unsubstituted aryl and a substituted aryl substituted with a substituent such as a halogen atom (e.g., a chlorine atom), an alkyl group (e.g., a methyl group) and an alkoxy group (e.g., a methoxy group)}, a nitro group, a hydroxy group, a halogen atom (e.g., a chlorine, bromine, or iodine atom), an alkoxy group (e.g., a methoxy or ethoxy group), and an amide group (i.e., an  $\text{NHCORo}$  group (Ro is an alkyl group having up to 8 carbon atoms)).

Suitable examples of compounds which can be used in the invention are given in the following without intending to limit the invention.

Compound 1



Compound 2Compound 3Compound 4Compound 5Compound 6Compound 7Compound 8

Compound 9

M.P. 247°C

Compound 10

M.P. 174°C

Compound 11

M.P. 238°C

Compound 12

M.P. 240°C

Compound 13

M.P. 156°C



-Continued

Compound 14Compound 15Compound 16Compound 17Compound 18

Compound 19Compound 20Compound 21Compound 22Compound 23

A general method of synthesis of the compound represented by the general formula is as follows:

## Synthesis Example 1 (Compound 5)

20.2 g of 4-phenylthiosemicarbazide was dissolved in 100 ml of pyridine and stirred with along with cooling with ice, added to ice water and the resulting crystals

60 were added to a 10% aqueous solution of sodium hydroxide followed by heating for 4 hours on a warm water bath. After the heating, the reaction solution was cooled and the solution made acidic with hydrochloric acid. The so obtained crystals were recrystallized from methanol to obtain 21.2 g of needle-like crystals melting at 103°C. 14.3 g of this crystal was dissolved in a solution of 2.6 g of sodium methylate dissolved in 150 ml

## 11

of methanol and stirred at room temperature (about 20° – 30°C). To this solution was added gradually dropwise at room temperature a solution of 9.6 g of 2,4-dinitrochlorobenzene dissolved in 100 ml of methanol. After the dropwise addition, the solution was heated for 2 hours on a warm water bath and concentrated to obtain crystals. These crystals were then recrystallized from methanol to obtain 15.4 g of yellow-white crystals having a melting point of 105°C.

Elementary Analysis for  $C_{21}H_{27}N_3O_5S$ 

|     |       |         |
|-----|-------|---------|
| C = | 58.74 | (58.85) |
| H = | 5.93  | (5.76)  |
| N = | 14.93 | (14.93) |

The numbers in the parentheses are the calculated values.

## Synthesis Examples 2 (Compound 18)

2.7 g of sodium methylate was added to 200 ml of absolute methanol and stirred under cooling with ice. To this solution was added gradually 8.3 g of 4-mercaptop-6-methyl-1,3,3a,7-tetrazaindene. Then 12.4 g of picryl chloride was dissolved in 150 ml of methanol and dropwise added gradually thereto at 0° – 5°C. After the dropwise addition, the solution was stirred for 2 hours under ice cooling and then allowed to stand at room temperature for one night. Yellow crystals were removed by filtration and recrystallized from a mixed solvent of ethanol and dimethylformamide thus to obtain 5 g of yellow crystals having a melting point of 165°C.

Analysis for  $C_{12}H_7N_3O_5S$ 

|     |       |         |
|-----|-------|---------|
| C = | 38.14 | (38.11) |
| H = | 1.80  | (1.86)  |
| N = | 26.20 | (25.99) |

The calculated values are shown in parentheses.

## Syntheses Example 3 (Compound 19)

8.2 g of 2-mercaptopbenzothiazole was dissolved in a solution of 2.7 g of sodium methylate dissolved in 200 ml of absolute methanol and stirred at room temperature. To this solution was dropwise added gradually a solution of 11 g of 2,4-dinitrochlorobenzene dissolved in 200 ml of methanol and thereafter, the mixture was stirred at room temperature for 2 hours. The so obtained crystals were recrystallized from a mixed solvent of benzene and ethanol (1:1 volume ratio) thus to obtain 5 g of yellow needlelike crystals having a melting point of 162°C.

Analysis for  $C_{13}H_7N_3O_5S_2$ 

|     |       |         |
|-----|-------|---------|
| C = | 46.83 | (46.85) |
| H = | 2.19  | (2.19)  |
| N = | 12.58 | (12.61) |

The calculated values are shown in parentheses.

As the emulsion of the type that is reversed using a compound represented by the general formula (I), a previously fogged silver halide emulsion is favorably used which does not have free electron trapping nuclei

## 12

in the interior of silver halide. An emulsion of this type is a silver halide emulsion consisting of normal crystals, preferably pure silver bromide, which has no twin surface and hardly has any crystal defects. This emulsion can further be improved with respect to the maximum density (Dmax), sensitization and clearness by the addition of bromide ions or iodide ions in an amount of from 1 to 20 mol %, preferably 3 to 10 mol %, of bromide or from 0.2 to 3 mol %, preferably from 0.5 to 2 mol %, of iodide per mole of silver. This emulsion does not provide directly a positive image by itself but a high reversal sensitization is provided by the incorporation of the nitrophenylmercapto group-containing heterocyclic compound of this invention. Examples of using an original emulsion having no electron trapping nuclei are described in British Pat. Nos. 1,186,717; 1,186,714 and 1,186,716; U.S. Pat. Nos. 3,501,306; 3,501,307; 3,501,310 and 3,531,288; French Pat. Nos. 1,520,821; 1,520,817; 1,522,354 and 1,520,824; and Belgian Pat. Nos. 795,354; 395,355; 395,359; 395,262 and 695,367.

Moreover, the nitrophenylmercapto group-containing heterocyclic compound used in this invention can also be used for the sensitization of a previously fogged silver halide photographic emulsion having free electron trapping nuclei in the interior of silver halide. In order to provide free electron trapping nuclei, it is desirable to use a chemical sensitizer or a salt of Group VIII metal as disclosed in, for example, U.S. Pat. Nos. 3,445,235; 3,537,858; 3,023,102 and 2,717,833; and British Pat. No. 707,704 during the formation of the silver halide precipitate. In addition, this emulsion can be improved by the addition of bromide ions or iodide ions with respect to the maximum density (Dmax), sensitization and clarity. Examples of the use of an original emulsion having electron trapping nuclei are described in Japanese Pat. No. Publications 4125/1968 and 29405/1968; U.S. Pat. Nos. 2,401,051, 2,717,833, 2,976,149, and 3,023,102; British Pat. Nos. 707,704, 1,097,999 and 690,997; French Pat. Nos. 1,520,822, 1,520,324, 1,520,817 and 1,523,626; Belgian Pat. Nos. 713,272, 721,567 and 681,768; and British Application No. 16,507,166.

The silver halide photographic emulsion used in the invention is previously fogged optically or chemically as disclosed in U.S. Pat. Nos. 2,497,875 and 3,537,858. The chemical fogging nuclei can be provided by the addition of organic reducing compounds, for example, hydrazine derivatives, formaldehyde, thiourea dioxide, a polyamine compound, an aminoborane and methylidichlorosilane.

The joint use of the reducing agent with metal more noble than silver or with a halide ion has been proposed as described in, for example, U.S. Pat. Nos. 2,497,875, 2,588,982, 3,023,102 and 3,367,778; British Pat. Nos. 707,704, 723,019, 821,251 and 1,097,999; French Pat. Nos. 1,513,840, 1,518,095, 1,498,213, 1,518,094, 1,520,822 and 1,520,824; Belgian Pat. Nos. 708,563 and 720,660; and Japanese Patent Publication 13488/1968. In the emulsion of the invention, gelatin is mainly used as a protective colloid and, in particular, an inert gelatin is preferably used. In place of the gelatin, photographically inert acylated gelatin derivatives such as phthalated gelatin, and water-soluble synthetic polymers such as polyvinyl acrylate, polyvinyl alcohol, polyvinylpyrrolidone and polyvinyl aginate can be used.

The silver halide emulsion according to the invention can also contain mercapto compounds, thione compounds and tetrazaindene compounds as a stabilizer for the fog nuclei as disclosed in U.S. Pat. Nos. 2,444,605; 2,444,606; 2,444,607 and 2,444,608; stilbene compounds and triazine compounds as a modifier of the clarity; chrome alum, 2,4-dichloro-s-triazine compounds, aziridine compounds, epoxy compounds and mucohalogenic acid compounds, halogenoformyl and maleic acid compounds as a brightening agent as disclosed in U.S. Pat. Nos. 3,406,070 and German Pat. Nos. 972,067 and 1,150,274, an ultraviolet ray absorbing agent and a hardener as disclosed in U.S. Pat. Nos. 3,288,775; 3,017,280 and 2,983,611; and British Pat. No. 1,167,207; sodium polyoxyalkylene sulfonates, saponins and anionic surface active agents having a betaine structure as a coating aid as disclosed in U.S. Pat. Nos. 2,600,831, 3,068,101 and 3,415,649; vinyl compounds such as polyalkyl acrylates and copolymers of an alkyl acrylate and acrylic acid, and polyalkylene oxide compounds as a preservative and plasticizer; and color couplers as disclosed in U.S. Pat. Nos. 2,376,679, 2,698,794, 3,046,129 and 3,227,554.

For these photographic emulsions, a spectrally sensitizing dye is used jointly with the nitrophenylmercapto group-containing heterocyclic compound. Suitable spectral sensitizers are dyes such as cyanines, merocyanines, composite trinuclear cyanines, composite trinuclear merocyanines, styryl dyes and hemicyanines.

In particular, a high sensitivity emulsion is obtained by the joint use of a dimethine dye such as is described in U.S. Pat. Applications Ser. Nos. 318,047, filed on Dec. 26, 1972; 351,386, filed Apr. 16, 1973; and 379,887, filed on July 16, 1973.

These emulsions can contain color couplers or can be developed with solutions containing couplers. Such color couplers can be incorporated in silver halide photographic emulsions for direct positives using suitable techniques as disclosed in U.S. Pat. Nos. 2,322,027, 2,801,171, 1,055,155, 1,102,028 and 2,186,849.

The grain size of silver halide in the photographic emulsion used in the invention is not limited, but the average grain size is preferably 0.05 to 1.0 microns. The form of the silver halide used can be either regular or irregular, but, in particular, the regular form is preferable. The effect of the invention is favourably provided by a monodispersed emulsion, although other emulsions than the monodispersed emulsion can, of course, be used.

The quantity of the nitrophenylmercapto group-containing heterocyclic compound used in the invention will vary depending upon the quantity of silver halide in the emulsion, the surface area and the end-use desired, and, preferably,  $1 \times 10^{-5}$  to  $5 \times 10^{-2}$  mol per 1 mol of the silver salt is generally employed. The nitrophenylmercapto group-containing heterocyclic compound is ordinarily added in the form of a solution in a suitable solvent such as water and organic solvents miscible with water, e.g., alcohols such as methanol and ethanol, ethers such as ethylene glycol monomethyl ether, ketones such as methyl ethyl ketone and acetone, N-containing compounds such as pyridine or mixtures of these solvents.

The addition of the nitrophenylmercapto group-containing heterocyclic compound to an emulsion is preferably carried out immediately before coating, but can be carried out during the chemical ageing or during the precipitating of the silver halide. The silver halide pho-

tographic emulsion for direct positives according to the instant invention is suitable for not only high contrast light-sensitive materials for direct positives, such as light-sensitive materials for lith-film copying originals, but also relatively low contrast light-sensitive materials for direct positives, such as light-sensitive materials for microphotographs or X-ray photographs. Moreover, it can be adapted to color light-sensitive materials, in particular, blue-sensitive layers, and, in addition to the use of light radiation, irradiation with electron rays, X-rays and  $\gamma$ -rays can also be used.

A first feature of the invention is to obtain a high reversal sensitivity within the blue range (e.g., about 400 to 500 nm) where a nitrophenylmercapto group-containing compounds used for sensitization. In particular, a phenylmercapto group-containing compound substituted with two nitro groups such as Compound 2 and Compound 6 described previously gives a high sensitivity. Where the heterocyclic ring of the general formula (I) is a 1,2,4-triazole ring, 1,3,3a,7-tetrazaindene or 7-tetrazaindene ring, in particular, a high sensitivity can be attained.

A second feature of the invention is that the nitrophenylmercapto group-containing heterocyclic compound used in the invention does not reduce the maximum density (D<sub>max</sub>) of an original emulsion.

A third feature of the invention is that a direct positive emulsion sensitized with the nitrophenylmercapto group-containing compound of the invention retains a predetermined maximum density and, simultaneously, retains a good clearness.

A fourth feature of the invention is that the nitrophenylmercapto group-containing heterocyclic compound used in the invention leaves substantially no residual color on a light-sensitive material after processing.

The nitrophenylmercapto group-containing heterocyclic compound of the invention can be used not only for the sensitization of previously fogged emulsions for direct positives, but also for various photographic objects in which a known desensitizer for silver halide photography is used. For example, (1) using an aqueous solution of the desensitizer as a pretreatment bath, a high sensitivity photographic material photographed is treated in this bath and developed while observing the progress of the development under a relatively bright illumination; (2) development is carried out in a mixed solution of the desensitizer and a developer used, whereby the sensitivity of a photographic light-sensitive material is reduced and the development can be accomplished under a relatively bright illumination; and (3) as described in Japanese Pat. Disclosure No. 3285/1972, the desensitizer can be used for an emulsion consisting of an internally latent image type silver halide doped with a multi-valent metal ion. Examples of suitable metal ions include Pb<sup>2+</sup>, Sb<sup>3+</sup>, As<sup>3+</sup>, Au<sup>3+</sup>, Bi<sup>3+</sup>, Rh<sup>3+</sup>, Pt<sup>4+</sup>, Os<sup>4+</sup>, Ir<sup>4+</sup> and Ir<sup>3+</sup> as disclosed in Japanese Patent Application Laid Open to Inspection No. 32813/72.

The following examples are given to illustrate the invention in greater detail without limiting the invention. Unless otherwise indicated, all parts, percents, ratios, etc., are by weight.

#### EXAMPLE 1

The method of preparing the emulsion used in this example was follows.

To a first solution prepared by adding 8 g of an inert gelatin to 5 ml of a 1 N solution of potassium bromide and 500 ml of water and warming to dissolve at 60°C were added a second solution prepared by adding 100 g of silver nitrate to 500 ml of water and warming to dissolve at 60°C and a third solution prepared by adding 70 g of potassium bromide to 150 ml of water and warming to dissolve at 60°C with stirring for a period of 50 minutes, and then the mixture was subjected to physical ageing for 5 minutes. Then 15 ml of a 0.2 N solution of potassium iodide was added and the pAg was adjusted to 6.0 using a solution of silver nitrate. Hydrazine (0.005 mm per mol of silver halide) and a chloroaurate (0.005 mm per mol of silver halide) were added to the mixture and the pH of the mixture was adjusted to 10 using a solution of sodium hydroxide, followed by ageing of the mixture. The mixture was then neutralized with citric acid, washed with water, melted and then mixed with a fourth solution prepared by dissolving 75 g of an inert gelatin in 300 ml of water to obtain a silver halide emulsion (original emulsion). The resulting emulsion had silver halide average grain size of about 0.2 micron in diameter and contained silver halide grains of normal tetragonal system having a (100) plane.

The compound of the invention was added to the above described original emulsion with 2.0 ml of an aqueous solution containing 1% by weight of saponin per kg of emulsion, and coated onto a film of cellulose triacetate to provide a thickness of 5 microns on dry basis. The coated specimen was exposed to a tungsten light at a color temperature of 2,854°K through an optical wedge, developed at 20°C for 2 minutes with the following developer, fixed to give a strip and the strip was then subjected to a measurement of the density using a P-type Densitometer manufactured by the Fuji Photo Film Co., Ltd. thus obtaining a characteristic curve. The results of sensitometry are shown in Table 1.

#### Composition of Developer

|                              |       |    |
|------------------------------|-------|----|
| Metol                        | 3.1   | g  |
| Anhydrous Sodium Sulfite     | 45    | g  |
| Hydroquinone                 | 12    | g  |
| Sodium Carbonate Monohydrate | 79    | g  |
| Potassium Bromide            | 2     | g  |
| Water to                     | 1,000 | ml |

This composition was used after being diluted with water in a proportion of 1:1 by volume.

In Table 1, the sensitivity is represented by the reciprocal of the exposure quantity E required to give a density of  $(D_{max} + D_{min})/2$  while setting the sensitivity of each comparative dye at 100 as a standard.  $D_{max}$  shows the maximum optical density and  $D_{min}$  shows the minimum optical density.

Table 1

| Test No. | Compound (molar concentration) ml/100 g emulsion | Sensitivity | D <sub>max</sub> | D <sub>min</sub> |
|----------|--------------------------------------------------|-------------|------------------|------------------|
| 1        | —                                                | —           | 2.2              | —                |
| 2        | 2 ( $8 \times 10^{-2}$ ) 16                      | 240         | 2.0              | 0.04             |
| 3        | 3 ( $8 \times 10^{-2}$ ) 32                      | 210         | 2.0              | 0.04             |
| 4        | 4 ( $8 \times 10^{-2}$ ) 32                      | 110         | 2.0              | 0.04             |
| 5        | 6 ( $8 \times 10^{-2}$ ) 16                      | 200         | 2.1              | 0.04             |
| 6        | 7 ( $8 \times 10^{-2}$ ) 32                      | 174         | 2.0              | 0.04             |
| 7        | 8 ( $8 \times 10^{-2}$ ) 16                      | 141         | 2.0              | 0.04             |
| 8        | 9 ( $8 \times 10^{-2}$ ) 16                      | 132         | 2.0              | 0.04             |
| 9        | 13 ( $8 \times 10^{-2}$ ) 16                     | 162         | 2.2              | 0.04             |
| 10       | 14 ( $8 \times 10^{-2}$ ) 64                     | 214         | 2.0              | 0.04             |

Table 1-continued

| Test No. | Compound (molar concentration) ml/100 g emulsion | Sensitivity | D <sub>max</sub> | D <sub>min</sub> |
|----------|--------------------------------------------------|-------------|------------------|------------------|
| 5        | 11 15 ( $8 \times 10^{-2}$ ) 16                  | 224         | 2.0              | 0.04             |
|          | 12 16 ( $8 \times 10^{-2}$ ) 32                  | 200         | 2.0              | 0.04             |
|          | 13 A ( $8 \times 10^{-2}$ ) 16                   | 100         | 1.3              | 0.05             |
|          | 14 A ( $8 \times 10^{-2}$ ) 24                   | 87          | 1.3              | 0.04             |
|          | 15 B ( $8 \times 10^{-2}$ ) 16                   | 89          | 2.2              | 0.23             |
|          | 16 B ( $8 \times 10^{-2}$ ) 24                   | 78          | 2.1              | 0.20             |
| 10       | 17 C ( $8 \times 10^{-2}$ ) 16                   | 46          | 2.2              | 0.05             |
|          | 18 C ( $8 \times 10^{-2}$ ) 24                   | 40          | 2.1              | 0.04             |

Compound A: Pinakryptol Yellow

Compound B: 3-Ethyl-5-m-nitrobenzilidene Rhodanine

Compound C: 5-m-Nitrobenzilidene Rhodanine

15 The Compounds A, B and C were used for comparison.

As is evident from the results in Table 1, the dyes represented by the general formula of the invention provide a direct positive silver halide emulsion having excellent photographic properties.

#### EXAMPLE 2

The method of preparing the emulsion used in this example was as follows.

25 To a first solution prepared by adding 10 g of an inert gelatin to 5 ml of a 1 N solution of sodium chloride and 500 ml of water and warming to dissolve at 60°C were added with agitation for a period of 20 minutes a second solution prepared by adding 100 g of silver nitrate to 500 ml of water and warming to dissolve at 60°C and a third solution prepared by adding 35 g of sodium chloride to 300 ml of water and warming to dissolve at 60°C.

35 After the addition, the mixture was aged for 5 minutes, mixed with agitation with a fourth solution prepared by adding 14 g of potassium bromide to 200 ml of water and warming to dissolve at 60°C, for a period of 20 minutes, then aged for 10 minutes, cooled and washed with water. After melting, the pH was adjusted to 10. Hydrazine and a chloroaurate, both in the proportion used in Example 1, were then added followed by ageing for 10 minutes and the pH was adjusted to 6.5 using citric acid. A fifth solution was prepared by dissolving 75 g of an inert gelatin in 300 ml of water and added to obtain a silver halide emulsion. The thus resulting silver halide emulsion (original emulsion) contained silver halide of an average grain size of about 0.15 micron in diameter.

40 To the above described original emulsion were added a 2-phenylindole nucleus-containing dimethine dye as shown in Table 2, a nitrophenylmercapto group-containing heterocyclic compound, 80 ml/kg-emulsion of a 10% aqueous solution of potassium bromide and 20 ml of an aqueous solution containing 1% by weight of saponin per kg of emulsion and 50 cc of an aqueous solution containing 2% by weight of mucochloric acid per kg of emulsion, and then the resulting emulsion was coated onto a film of cellulose triacetate to provide a thickness of 2 microns on dry basis. The coated specimen was exposed to a tungsten light at a color temperature of 2,854°K through an optical wedge, developed at 20°C for 3 minutes with a developer consisting mainly of a polyhydroxybenzene as described in Example 1, fixed to give a strip and the strip was then subjected to a measurement of the density using a P-type Densitometer manufactured by the Fuji Photo Film Co., Ltd. thus obtaining a characteristic curve. The results of the sensitometry are shown in Table 2.

Table 2

| Test No. | Dye (molar concentration)<br>ml/100 g emulsion | Compound (molar concentration)<br>ml/100 g emulsion | Sensitivity | D <sub>max</sub> | D <sub>min</sub> |
|----------|------------------------------------------------|-----------------------------------------------------|-------------|------------------|------------------|
| 1        | I (8 × 10 <sup>-3</sup> ) 8                    |                                                     | 100         | 3.0              | 0.15             |
| 2        | "                                              | 2 (8 × 10 <sup>-3</sup> ) 32                        | 409         | 2.74             | 0.04             |
| 3        | "                                              | 3 (8 × 10 <sup>-3</sup> ) 64                        | 324         | 3.0              | 0.04             |
| 4        | II (8 × 10 <sup>-3</sup> ) 16                  | —                                                   | 100         | 3.5              | 0.14             |
| 5        | "                                              | 4 (8 × 10 <sup>-3</sup> ) 64                        | 245         | 3.16             | 0.04             |
| 6        | "                                              | 6 (8 × 10 <sup>-3</sup> ) 64                        | 264         | 3.38             | 0.04             |
| 7        | III (8 × 10 <sup>-3</sup> ) 8                  | —                                                   | 100         | 3.5              | 0.12             |
| 8        | "                                              | 7 (8 × 10 <sup>-3</sup> ) 64                        | 129         | 3.46             | 0.05             |
| 9        | "                                              | 8 (8 × 10 <sup>-3</sup> ) 32                        | 118         | 3.30             | 0.04             |
| 10       | IV (8 × 10 <sup>-3</sup> ) 16                  | —                                                   | 100         | 3.4              | 0.14             |
| 11       | "                                              | 2 (8 × 10 <sup>-3</sup> ) 32                        | 398         | 3.4              | 0.04             |
| 12       | "                                              | 8 (8 × 10 <sup>-3</sup> ) 64                        | 372         | 3.4              | 0.04             |
| 13       | V (8 × 10 <sup>-3</sup> ) 32                   | —                                                   | 100         | 3.5              | 0.15             |
| 14       | "                                              | 2 (8 × 10 <sup>-3</sup> ) 16                        | 381         | 3.4              | 0.04             |
| 15       | "                                              | 8 (8 × 10 <sup>-3</sup> ) 32                        | 372         | 3.5              | 0.04             |

Dye I



Dye II



Dye III



Dye IV



Dye V



30

As is evident from the results contained in Table 2, a silver halide photographic emulsion for direct positives, which has a higher sensitivity and greatly improved clearness, is provided by the combination of the compound represented by the general formula of the invention with a sensitizer.

While the invention has been described in detail and with reference to specific embodiments thereof, it will be apparent to one skilled in the art that various changes and modifications can be made therein without departing from the spirit and scope thereof.

What is claimed is:

1. A silver halide photographic emulsion for direct positives, containing fogged silver halide grains and an amount of at least one compound sufficient for sensitization in the blue color region represented by the general formula (1)

50



60

in which Z represents a group of non-metallic atoms necessary for forming a heterocyclic ring selected from the group consisting of a 1,2,4-triazole ring, a 1,3,4-thiadiazole ring, a 1,3,3a,7-tetraazaindene ring, a benzothiazole ring, a benzimidazole ring and a pyrimidine ring, and n represents an integer of from 1 to 3.

2. The silver halide photographic emulsion of claim 1, wherein said heterocyclic ring is a 1,2,4-triazole ring.

19

3. The silver halide photographic emulsion of claim 1, wherein said heterocyclic ring is a 1,3,3a,7-tetrazain-dene ring.

4. The silver halide photographic emulsion of claim 1, wherein said heterocyclic ring is a 1,3,4-thiadiazole ring.

5. The silver halide photographic emulsion of claim 1, wherein said heterocyclic ring is a pyrimidine ring.

6. The silver halide photographic emulsion of claim 1, wherein said heterocyclic ring is a benzothiazole ring.

7. The silver halide photographic emulsion of claim 1, wherein said heterocyclic ring is a benzoimidazole ring.

8. The silver halide photographic emulsion of claim 1, wherein said silver halide grains are chemically fogged.

9. The silver halide photographic emulsion of claim 8, wherein said silver halide grains are fogged with a reducing agent and a gold compound.

10. The silver halide photographic emulsion of claim 1, wherein said emulsion contains a photographic color coupler.

11. The silver halide photographic emulsion of claim 1, wherein said emulsion contains a spectral sensitizer.

12. The silver halide photographic emulsion of claim 1, wherein said compound is



3,910,795

**21**

-Continued



5



15



30



45



60

**22**

25



35



50



55



65

23

-Continued



or



13. A silver halide photographic material for direct positives, comprising a support having coated thereon 30 the silver halide photographic emulsion of claim 1.

14. The silver halide photographic material of claim 13, wherein said heterocyclic ring is a 1,2,4-triazole ring.

15. The silver halide photographic material of claim 13, wherein said heterocyclic ring is a 1,3,3a,7-tetraazaindene ring.

16. The silver halide photographic material of claim 13, wherein said heterocyclic ring is a 1,3,4-thiadiazole ring.

17. The silver halide photographic material of claim 13, wherein said heterocyclic ring is a pyrimidine ring.

18. The silver halide photographic material of claim 13, wherein said heterocyclic ring is a benzothiazole ring.

19. The silver halide photographic material of claim 13, wherein said heterocyclic ring is a benzoimidazole ring.

20. The silver halide photographic material of claim 13, wherein said silver halide grains are chemically 50 fogged.

21. The silver halide photographic material of claim 20, wherein said silver halide grains are fogged with a reducing agent and a gold compound.

22. The silver halide photographic material of claim 13, wherein said emulsion contains a photographic color coupler.

23. The silver halide photographic material of claim 13, wherein said emulsion contains a spectral sensitizer.

24. The silver halide photographic material of claim 13, wherein said compound is



24





5



10



20



30



40



50



27  
-Continued



28



10 OR



20

30

35

40

45

50

55

60

65